

# UNITED STATES PATENT OFFICE.

GEORGE FRANCOIS JAUBERT, OF PARIS, FRANCE.

## MANUFACTURE OF ALLOYS OF THE ALKALI METALS.

SPECIFICATION forming part of Letters Patent No. 709,489, dated September 23, 1902.

Application filed February 23, 1901. Serial No. 48,415. (No specimens.)

To all whom it may concern:

Be it known that I, GEORGE FRANCOIS JAUBERT, a citizen of the Republic of Switzerland, residing at Paris, in the Republic of France, have invented certain new and useful Improvements in the Manufacture of Alloys of the Alkaline Metals, of which the following is a specification.

I have found that if under certain conditions potassium is caused to react upon caustic soda or sodium upon caustic potash liquid alloys of potassium and sodium are obtained containing about eighty per cent. of potassium.

15 Example I: Four parts of well-dried caustic soda and twelve parts of metallic potassium are melted in a suitable crucible, which is heated on an oil-bath which is provided with means for forming a vacuum. At between about 200° to 250° centigrade a moderately brisk reaction is observed. The temperature is further raised to about 300° centigrade and the mixture then allowed to cool. There is found at the bottom of the vessel a 25 layer of caustic alkali and above it a liquid residue, which is decanted and preserved under petroleum. Analysis shows that this residue contains about seventy-seven per cent. of potassium and twenty-three per cent. of sodium and corresponds pretty exactly to the formula  $\text{NaK}_2$ .

Example II: A mixture of eight parts of caustic potash and five parts of sodium is heated on an oil-bath *in vacuo*. At about 225° centigrade there is a very brisk reaction and the operation may perhaps be considered as at an end; but for greater security it is nevertheless heated to about 250° to 275° centigrade and is then allowed to cool and the alloy formed is decanted. This alloy corresponds in a large degree to the formula  $\text{NaK}$ , for it contains about sixty-three per cent. of potassium and thirty-seven per cent. of sodium.

45 The alloys obtained in Examples I and II

are liquid at the ordinary temperature and resemble mercury. They are much lighter than water and float upon heavy petroleum. They are eminently oxidizable and even in the cold become covered with a black coating 50 of oxid. They react in many cases in which sodium is inert.

The proportions of sodium and of potassium may vary in the alloy according to the formulas used. Thus



Again,



Having thus described the nature and object of my invention, what I claim as new, and desire to secure by Letters Patent, is—

1. The method of manufacturing alloys of the alkali metals, such as potassium and sodium, which consists in mixing one of the metals with a caustic oxid of the other metal, 70 then heating the mixture *in vacuo* at a temperature of from 200° to 300° centigrade, and in then allowing the residue to cool, substantially as and for the purposes described.

2. The method of manufacturing an alloy 75 of the alkali metals, which consists in mixing potassium with caustic soda in required proportions, then heating the mixture in substantial *vacuo* at a temperature of from 200° to 300° centigrade, and in finally cooling the 80 residue, substantially as and for the purposes described.

In testimony whereof I have signed this specification in the presence of two subscribing witnesses.

GEORGE FRANCOIS JAUBERT.

Witnesses:

C. DE MESTRAL,

EDWARD P. MACLEAN.